

3,442,653  
SENSITIZED SILVER HALIDE SYSTEMS  
WITH ACTIVATED NONLABILE SELENIUM COMPOUNDS

Joseph S. Dunn, Rochester, N.Y., assignor to Eastman Kodak Company, Rochester, N.Y., a corporation of New Jersey

No Drawing. Continuation-in-part of application Ser. No. 468,972, July 1, 1965. This application Mar. 29, 1968, Ser. No. 717,396

Int. Cl. G03c 1/50, 1/10

U.S. Cl. 96—108

15 Claims

## ABSTRACT OF THE DISCLOSURE

Sensitizing photographic systems such as a silver halide emulsion with a noble metal and labile selenium formed in situ by activating a non-labile selenium compound. Specific activation methods include the use of reducing agents.

This application is a continuation-in-part of my co-pending application Ser. No. 606,587 filed Jan. 3, 1967, now abandoned, which is a continuation-in-part of my application Ser. No. 468,972 filed July 1, 1965, now U.S. Patent No. 3,297,446 which in turn was a continuation-in-part of Ser. No. 343,465 filed Feb. 10, 1964, now abandoned.

This invention relates to photography. In one aspect, this invention relates to processes of sensitizing photographic systems.

In my earlier-filed application Ser. No. 468,972, now U.S. Patent 3,297,446, I found that a sensitizer combination of a noble metal and labile selenium produced a synergistic effect in photographic systems. There are many readily available selenium compounds which are not labile, however, and it would be desirable to employ these compounds in a sensitizing process. The invention provides a way for employing these compounds in such a sensitizing process.

It is an object of this invention to provide a process for sensitizing photographic systems with a noble metal and labile selenium wherein a non-labile selenium compound is employed in the process.

Another object of this invention is to provide a process for sensitizing photographic silver halide emulsions with a noble metal and labile selenium wherein a non-labile selenium compound is employed in the process.

Still another object of this invention is to provide a process for sensitizing photographic systems and more particularly silver halide emulsions with gold and labile selenium wherein a non-labile selenium compound is employed in the process.

Yet still another object of the invention is to provide a sensitizing process for photographic systems which can be easily controlled.

Other objects will become apparent hereinafter.

These and other objects of the invention are accomplished by sensitizing photographic systems and more particularly silver halide emulsions with a noble metal and labile selenium which is formed in situ by activating a non-labile selenium compound. It was previously thought that non-labile selenium compounds could not be employed in combination with noble metals in a sensitizing process for photographic systems. I have found, however, that non-labile selenium compounds can be activated so that they become labile and, in combination with noble metals, give synergistic sensitization.

A unique feature of using the sensitizing process of this invention is that sensitization of photographic systems can be easily controlled. Sensitization can occur

whenever desired by activating the non-labile selenium compound at that time. The degree of sensitization can also be controlled by varying the intensity of activation. A predetermined sensitivity of a photographic system can thus be obtained with the sensitizing process of this invention.

Any method for activating non-labile selenium compounds can be used in this invention so long as it renders the selenium compounds labile. A preferred way of activating non-labile selenium compounds to make them labile is by employing reducing agents. Other methods for activating non-labile selenium compounds to make them labile are disclosed and claimed in copending application Ser. Nos. 606,586 and 606,588 both entitled "Sensitizing Photographic Systems" of my co-worker McVeigh filed concurrently herewith.

The term "labile" has a meaning well understood by those skilled in the art of photography and is defined in my earlier-filed application Ser. No. 468,972, filed July 1,

20 1965 now U.S. Patent 3,297,446, as being a material which yields a silver selenide that is insoluble in water at room temperature (20° C.) upon addition to an aqueous silver nitrate solution. Likewise, the term "non-labile" as used herein in describing selenium compounds has a meaning well understood by those skilled in the art of photography, i.e., a material which does not yield a silver selenide that is insoluble in water at room temperature (20° C.) upon addition to an aqueous silver nitrate solution. For example, potassium selenocyanate and selenous acid are non-labile selenium compounds since silver selenide does not precipitate when these compounds are added to an aqueous silver nitrate solution.

Non-labile selenium compounds which can be used in this invention include, for example, potassium selenocyanate, selenous acid, inorganic isoselenocyanate complexes, etc.

The concentration of the non-labile selenium compound which is activated to form labile selenium in situ can be varied considerably depending upon the particular non-labile selenium compound employed, the nature of the photographic system, the amount and chemical nature of the noble metal sensitizer, etc. In silver halide systems, for example, I have found that useful results can be obtained using amounts as small as 0.05 mg. of non-labile selenium compound per mole of silver halide although considerably larger amounts can also be employed, such as 5.0 mg. or more per mole of silver halide.

The noble metal sensitizers useful in my invention include the well-known gold sensitizers and other noble metals such as palladium, platinum and any of those disclosed in Smith et al., U.S. Patent No. 2,448,060, issued Aug. 31, 1948. Typical suitable gold sensitizers are described in Waller et al., U.S. Patent No. 2,399,083, issued Apr. 23, 1946, and Damschroder et al., U.S. Patent 2,642,361, issued June 16, 1953.

Illustrative addenda suitable for furnishing the noble metal moiety in the sensitizer combinations of the invention include:

60 gold chloride,  
potassium aurate,  
potassium auraurite,  
potassium auricyanide,  
potassium aurithiocyanate,  
65 gold sulfide,  
gold selenide,  
gold iodide,  
potassium chloroaurate,  
70 ethylenediamine-bis-gold chloride,  
ammonium chloroplatinite, i.e.  $(\text{NH}_4)_2\text{PtCl}_4$ ,  
ammonium chloropalladate, i.e.  $(\text{NH}_4)_2\text{PdCl}_6$ ; and



a rather high degree of polarity are preferred. Where it is desired to add the sensitizing addenda in some other form than a solution, this procedure is also possible, especially where the sensitizer is available in the form of a colloidal suspension. In some cases, it is possible to add the sensitizers suspended in an organic solvent which forms very small suspended particles in the photographic emulsion similar to the type of colloidal particle produced in preparing coupler dispersions. Dispersing media useful for this purpose include tricresyl phosphate, dibutyl phthalate, triphenyl phosphate, etc.

Vacuum deposited photographic systems substantially free of conventional vehicles, binders or dispersing agents can also be sensitized in accordance with the invention by incorporating the sensitizers, before or after activation, in a coating or layer contiguous to the vacuum deposited light-sensitive material. Suitable vacuum deposited silver halide systems that can be sensitized in accordance with the invention are disclosed in Rasch et al. application U.S. Ser. No. 415,596 filed Dec. 3, 1964; Rees application U.S. Ser. No. 421,725 filed Dec. 28, 1964 now U.S. Patent 3,384,490; and Belgian Patent 639,020.

The silver halide emulsion of a photographic element which can be sensitized according to this invention can contain conventional addenda such as gelatin plasticizers, coating aids, antifoggants such as the azaindines and hardeners such as aldehyde hardeners, e.g., formaldehyde, mucochloric acid, glutaraldehyde bis(sodium bisulfite), maleic dialdehyde, aziridines, dioxane derivatives and oxy-polysaccharides. The addenda may be added to the emulsion before or after sensitizing dyes, if any, are used. Sensitizing dyes useful in sensitizing such emulsions are described, for example, in U.S. Patents 2,526,632 and 2,503,776. Spectral sensitizers which can be used are the cyanines, merocyanines, complex (trinuclear) cyanines, complex (trinuclear) merocyanines, styryls and hemicyanines. Developing agents can also be incorporated into the silver halide emulsion if desired or can be contained in a separate underlayer. Various silver salts may be used as the sensitive salt such as silver bromide, silver iodide, silver chloride, or mixed silver halides such as silver chlorobromide or silver bromoiodide.

The silver halide emulsion layer of a photographic element which can be sensitized according to the instant invention can contain any of the hydrophilic water-permeable binding materials suitable for this purpose. Suitable materials include gelatin, colloidal albumin, polyvinyl compounds, cellulose derivatives, acrylamide polymers, etc. Mixtures of these binding agents can also be used. The binding agents for the emulsion layer of the photographic element can also contain dispersed polymerized vinyl compounds. Such compounds are disclosed, for example, in U.S. Patents 3,142,568; 3,193,386; 3,062,674; and 3,220,844, and include the water-insoluble polymers of alkyl acrylates and methacrylates acrylic acid, sulfoalkyl acrylates or methacrylates and the like.

The silver halide emulsion of a photographic element which can be sensitized according to the instant invention may be coated on a wide variety of supports. Typical supports are cellulose nitrate film, cellulose ester film, polyvinyl acetal film, polystyrene film, poly(ethylene terephthalate) film and related films or resinous materials as well as glass, paper, metal and the like. Supports such as paper which are coated with  $\alpha$ -olefin polymers, particularly polymers of  $\alpha$ -olefins containing two or more carbon atoms, as exemplified by polyethylene, polypropylene, ethylene-butene copolymers and the like can also be employed.

I have found that the speed of photographic emulsions sensitized according to the invention can be further increased by including in the emulsions a variety of hydrophilic colloids, such as carboxymethyl protein of the type described in U.S. Patent 3,011,890, issued Dec. 5, Canadian Patent 635,206.

Photographic emulsions sensitized according to the in-

vention can contain speed increasing compounds such as quaternary ammonium compounds, polyethylene glycols or thioethers. Frequently, useful effects can be obtained by adding the aforementioned speed increasing compounds to the photographic developer solutions instead of, or in addition to, the photographic emulsions.

The sensitizing process of the invention can be used for various kinds of photographic systems. In addition to being useful in X-ray and other nonoptically sensitized systems, they can also be used in orthochromatic, panchromatic, and infrared sensitive systems. The sensitizing addenda can be added to photographic systems before or after any sensitizing dyes which are used.

The sensitizing process of the invention can be used in emulsions intended for color photography, for example, emulsions containing color-forming couplers or emulsions to be developed by solutions containing couplers or other color-generating materials, emulsions of the mixed-packet type, such as described in Godowsky U.S. Patent 2,698,794 issued Jan. 4, 1955; in silver dye-bleach systems; and emulsions of the mixed-grain type, such as described in Carroll and Hanson U.S. Patent 2,592,243, issued Apr. 8, 1952.

The sensitizing process of the invention can be utilized to sensitize any photographic system that can be sensitized with noble metals. The invention thus has utility, not only for silver halide photographic systems, but also for other light-sensitive systems such as other light-sensitive silver salts, thallous halides, cuprous halides, lead halides and related light-sensitive heavy metal salts.

Photographic elements which have been sensitized according to the process of the instant invention may be stabilized with labile sulfur compounds in accordance with application Ser. No. 486,235 of McVeigh filed Sept. 9, 1965, now U.S. Patent 3,297,447. These labile sulfur compounds provide a particularly efficacious means of controlling fog without deleteriously affecting the speed of the stabilized photographic system. Particularly useful labile sulfur compounds include the water-soluble thiosulfates such as alkali metal thiosulfates including sodium and potassium thiosulfates, as well as ammonium thiosulfate; thioureas such as thiourea, allylisothiourea, diacetyl thiourea; thiosemicarbazide; thiocarbamates such as isopropylthiocarbamate; etc.

The amount of labile sulfur compound used to stabilize photographic systems sensitized by the process of this invention can vary considerably depending upon the particular sensitized photographic system employed, finishing conditions, including temperature and time of digestion and ripening, etc. In silver halide photographic systems, particularly useful results have been obtained at concentrations of about 0.1 to 10 mg. per mole of silver halide. Larger or smaller quantities can be employed without adversely affecting the sensitometric properties of the photographic system. The labile sulfur compounds are efficaciously added to be present during the chemical sensitization of the photographic system.

The following examples will illustrate the invention but are not to be construed to limit it in any way.

#### EXAMPLE 1

##### Activation by reducing agents

A medium grain silver bromoiodide emulsion containing 3.4 mole percent iodide is prepared. A first portion of the emulsion is chemically sensitized by the addition of 2 mg. of potassium chloroaurate per silver mole, 100 mg. of potassium thiocyanate per silver mole and 1.6 mfi. of potassium selenocyanate per silver mole. The emulsion is then heated for 40 minutes at 65° C.

A second portion of the emulsion is sensitized in the same manner as the first portion but with the addition of 10.1 mg. of benzothiazole methiodide per silver mole and heating for 9 minutes at 65° C.

A third portion of the emulsion is sensitized in the

same manner as the first portion except for the addition of 8.2 mg. of benzothiazole methbromide per silver mole and heating for 9 minutes at 65° C.

A fourth portion of the emulsion is sensitized in the same manner as the first portion except for the addition of 11.7 mg. of 2-hydroxymethylbenzothiazole ethyliodide per silver mole and heating for 12 minutes at 65° C.

These emulsions are then coated on a cellulose acetate support at a coverage of 540 mg. of silver per square foot. The coatings are then exposed on an intensity scale sensitometer, processed for 5 minutes in Kodak Developer DK-50, fixed, washed and dried.

The following results are obtained:

| Portion | Reducing agent                           | Relative speed | Fog  |
|---------|------------------------------------------|----------------|------|
| First   | None                                     | 100            | 0.03 |
| Second  | Benzothiazole methiodide                 | 229            | 0.11 |
| Third   | Benzothiazole methbromide                | 240            | 0.21 |
| Fourth  | 2-hydroxymethyl-benzothiazole methiodide | 204            | 0.27 |

This example shows that reducing agents activate potassium selenocyanate to make it labile with an increase in speed of up to 140%.

#### EXAMPLE 2

##### Activation by other reducing agents

A first portion of the emulsion of Example 1 is chemically sensitized with 2 mg. of potassium chloroaurate per silver mole, 100 mg. of potassium thiocyanate per silver mole and 1.6 mg. of potassium selenocyanate per silver mole. The sensitized emulsion is then heated for 40 minutes at 65° C.

A second portion of the emulsion is chemically sensitized with 4 mg. of potassium chloroaurate per silver mole, 100 mg. of potassium thiocyanate per silver mole, 1.6 mg. of potassium selenocyanate per silver mole and 20.2 mg. of benzothiazole methiodide per silver mole. This portion is then heated for 15 minutes at 65° C.

A third portion of the emulsion is sensitized in the same manner as the second portion except that the benzo-

per silver mole. The emulsion is then heated for 30 minutes at 60° C.

A second portion of the emulsion is sensitized in the same manner as the first portion except for the addition of 2.8 mg. of triphenylphosphine per silver mole and heating for 6 minutes at 60° C.

A third portion of the emulsion is sensitized in the same manner as the first portion except for the addition of 10.1 mg. of benzothiazole methiodide per silver mole and heating for 20 minutes at 60° C.

These emulsions are then coated and processed in the same manner as in Example 1 with the following results:

| Portion | Reducing agent           | Relative speed | Fog  |
|---------|--------------------------|----------------|------|
| First   | None                     | 10             | 0.02 |
| Second  | Triphenylphosphine       | 100            | 0.06 |
| Third   | Benzothiazole methiodide | 100            | 0.03 |

This example shows that reducing agents convert a non-labile selenium compound into a labile form which is an effective sensitizer.

#### EXAMPLE 4

##### Equivalence of labile selenium sensitizers with activated non-labile selenium compounds

A first portion of the emulsion of Example 1 is chemically sensitized with 2 mg. of potassium chloroaurate per silver mole, 100 mg. of potassium thiocyanate per silver mole and 0.8 mg. of N,N-dimethylselenourea per silver mole. The sensitized emulsion is then heated for 15 minutes at 65° C.

A second portion of this emulsion is chemically sensitized with 4 mg. of potassium chloroaurate per silver mole, 100 mg. of potassium thiocyanate per silver mole, 1.6 mg. of potassium selenocyanate per silver mole and 20.2 mg. of benzothiazole methiodide per silver mole. This portion of the emulsion is also heated for 15 minutes at 65° C.

These emulsions are then coated and processed in the same manner as in Example 1 with the following results:

| Portion | Sensitizers                                      | Reducing agent           | Relative speed | Fog  |
|---------|--------------------------------------------------|--------------------------|----------------|------|
| First   | Potassium chloroaurate-N,N-dimethylselenourea.   | None                     | 1,000          | 0.21 |
| Second  | Potassium chloroaurate-Po-tassium selenocyanate. | Benzothiazole methiodide | 970            | 0.17 |

This example shows that non-labile compounds which are activated by reducing agents are equivalent in their sensitizing action to labile selenium compounds.

#### EXAMPLE 5

##### Equivalence of labile selenium sensitizers with activated non-labile selenium compounds

A first portion of the emulsion of Example 1 is chemically sensitized with 100 mg. of potassium thiocyanate per silver mole and 0.8 mg. of N,N-dimethylselenourea per silver mole. This emulsion is then heated for 9 minutes at 60° C.

A second portion of this emulsion is sensitized with 100 mg. of potassium thiocyanate per silver mole, 1.6 mg. of potassium selenocyanate per silver mole and 1.4 mg. of triphenylphosphine per silver mole. This emulsion is then heated for 6 minutes at 60° C.

These emulsions are then coated and processed in the same manner as in Example 1 with the following results:

| Portion | Reducing agent           | Relative speed | Fog  |
|---------|--------------------------|----------------|------|
| First   | None                     | 100            | 0.03 |
| Second  | Benzothiazole methiodide | 302            | 0.17 |
| Third   | 2-mercaptopbenzoic acid  | 289            | 0.20 |

#### EXAMPLE 3

##### Activation by reducing agents in the absence of a noble metal

A first portion of the emulsion of Example 1 is chemically sensitized with 100 mg. of potassium thiocyanate per silver mole and 1.6 mg. of potassium selenocyanate

| Portion | Sensitizer              | Reducing agent     | Relative speed | Fog  |
|---------|-------------------------|--------------------|----------------|------|
| First   | N,N-dimethyl selenourea | None               | 500            | 0.03 |
| Second  | Potassium selenocyanate | Triphenylphosphine | 450            | 0.06 |

## EXAMPLE 6

Synergistic effect of reducing agent with non-labile selenium compound

A first portion of the emulsion of Example 1 is sensitized with 100 mg. of potassium thiocyanate per silver mole and 2.8 mg. of triphenylphosphine per silver mole. This emulsion is then heated for 30 minutes at 60° C.

A second portion of the emulsion is sensitized with 100 mg. of potassium thiocyanate per silver mole and 1.6 mg. of potassium selenocyanate per silver mole and then heated for 30 minutes at 60° C.

A third portion of the emulsion is sensitized in the same manner as the first portion but the addition of 1.6 mg. of potassium selenocyanate per silver mole and heating for 6 minutes at 60° C.

| Portion     | Sensitizer                                 | Reducing agent      | Relative speed | Gamma | Fog  |
|-------------|--------------------------------------------|---------------------|----------------|-------|------|
| First.....  | Sodium thiosulfate-potassium chloroaurate. | None.....           | 750            | 0.93  | 0.14 |
| Second..... | Selenous acid potassium chloroaurate.....  | Sodium sulfite..... | 1,000          | 1.03  | 0.14 |

These emulsions are then coated and processed in the same manner as in Example 1 with the following results:

| Portion     | Compound added                              | Relative speed | Fog  |
|-------------|---------------------------------------------|----------------|------|
| First.....  | Triphenylphosphine.....                     | 10             | 0.02 |
| Second..... | Potassium selenocyanate.....                | 100            | 0.03 |
| Third.....  | Triphenylphosphine-potassium selenocyanate. | 100            | 0.06 |

This example illustrates the synergistic effect which is obtained when a reducing agent is combined with a non-labile selenium compound. An increase in speed of 1000% is obtained.

| Portion      | Sensitizer                                                                  | Reducing agent | Relative speed | Gamma | Fog  |
|--------------|-----------------------------------------------------------------------------|----------------|----------------|-------|------|
| First.....   | None.....                                                                   | 30             | <1             | 0.80  | 0.03 |
| Second.....  | Selenous acid (3.27) (non-labile selenium compound).                        | 30             | 24             | 0.37  | 0.03 |
| Third.....   | Sodium sulfite (6.3) (reducing agent).                                      | 30             | <1             | 0.12  | 0.03 |
| Fourth.....  | Potassium chloroaurate (1.0).                                               | 25             | 24             | 0.28  | 0.08 |
| Fifth.....   | Selenous acid (3.27) + Potassium chloroaurate (1.0).                        | 30             | 25             | 0.28  | 0.09 |
| Sixth.....   | Sodium sulfite (6.3) + Potassium chloroaurate (1.0).                        | 30             | 12             | 0.22  | 0.13 |
| Seventh..... | Selenous acid (3.27) + Sodium sulfite (6.3).                                | 10             | 250            | 1.42  | 0.18 |
| Eighth.....  | Selenous acid (3.27) + Sodium sulfite (6.3) + Potassium chloroaurate (1.0). | 25             | 1,000          | 1.68  | 0.20 |

## EXAMPLE 7

## Effect of reducing agents on labile selenium compounds

A first portion of the emulsion of Example 1 is chemically sensitized with 2 mg. of potassium chloroaurate per silver mole, 100 mg. of potassium thiocyanate per silver mole and 0.8 mg. of N,N-dimethyl selenourea per silver mole. This emulsion is then heated for 15 minutes at 65° C.

A second portion of the emulsion is sensitized in the same manner as the first portion except that 10.1 mg. of benzothiazole methiodide per silver mole are added. The second portion is then heated for 30 minutes at 65° C.

These emulsions are then coated and processed in the same manner as in Example 1 with the following results:

| Portion     | Sensitizer                                      | Reducing agent            | Relative speed | Fog  |
|-------------|-------------------------------------------------|---------------------------|----------------|------|
| First.....  | Potassium chloroaurate-N-N-dimethyl selenourea. | None.....                 | 1,000          | 0.21 |
| Second..... | Potassium chloroaurate-N,N-dimethyl selenourea. | Benzothiazole methiodide. | 950            | 0.17 |

This example shows that reducing agents have no effect on selenium compounds which are already labile (N,N-

dimethyl selenourea is disclosed as being labile in my earlier filed application Ser. No. 468,972, filed July 1, 1965, now U.S. Patent 3,297,446).

## EXAMPLE 8

## 5 Comparison of activated non-labile selenium compounds with conventional sensitizers

An emulsion similar to that of Example 1 is prepared and sensitized with 2.0 mg. of sodium thiosulfate per silver mole and 0.75 mg. of potassium chloroaurate per silver mole. A second portion of the emulsion is sensitized with 49 mg. of selenous acid per silver mole, 94.6 mg. of sodium sulfite per silver mole and 0.75 mg. of potassium chloroaurate per silver mole. These emulsions are then coated and processed in the same manner as in Example 1 with the following results:

10

15

20

25

30

This example shows that gold and non-labile selenium compounds which have been made labile with reducing agents are better sensitizers than conventional sulfur and gold sensitizers.

## EXAMPLE 9

## Synergistic effect of reducing agent with non-labile selenium compound

Portion of an emulsion similar to that of Example 1 are sensitized with various sensitizers as set forth below. These emulsions are then coated and processed in the same manner as in Example 1 with the following results:

30

| Portion      | Sensitizer                                                                  | Reducing agent | Relative speed | Gamma | Fog  |
|--------------|-----------------------------------------------------------------------------|----------------|----------------|-------|------|
| First.....   | None.....                                                                   | 30             | <1             | 0.80  | 0.03 |
| Second.....  | Selenous acid (3.27) (non-labile selenium compound).                        | 30             | 24             | 0.37  | 0.03 |
| Third.....   | Sodium sulfite (6.3) (reducing agent).                                      | 30             | <1             | 0.12  | 0.03 |
| Fourth.....  | Potassium chloroaurate (1.0).                                               | 25             | 24             | 0.28  | 0.08 |
| Fifth.....   | Selenous acid (3.27) + Potassium chloroaurate (1.0).                        | 30             | 25             | 0.28  | 0.09 |
| Sixth.....   | Sodium sulfite (6.3) + Potassium chloroaurate (1.0).                        | 30             | 12             | 0.22  | 0.13 |
| Seventh..... | Selenous acid (3.27) + Sodium sulfite (6.3).                                | 10             | 250            | 1.42  | 0.18 |
| Eighth.....  | Selenous acid (3.27) + Sodium sulfite (6.3) + Potassium chloroaurate (1.0). | 25             | 1,000          | 1.68  | 0.20 |

This example shows that activating a non-labile selenium compound with a reducing agent will increase the relative speed of an emulsion by over 1000%. This example also shows that the addition of a gold compound plus a reducing agent to a non-labile selenium compound will increase the relative speed of an emulsion by over 4000%.

60

## EXAMPLE 10

A first portion of an emulsion similar to that of Example 1 is chemically sensitized with 4 mg. of potassium chloroaurate per silver mole, 100 mg. of sodium thiocyanate per silver mole, 1.6 mg. of potassium selenocyanate per silver mole and 20.2 mg. of benzothiazole methiodide

per silver mole and is then heated for 15 minutes at 65° C.

## 11

A second portion of the emulsion is chemically sensitized in the same manner as the first portion but with the addition of 4 mg. of sodium thiosulfate per silver mole and heating for 10 minutes at 60° C.

| Portion | Sensitizer         | Relative speed | Fog  |
|---------|--------------------|----------------|------|
| First   | None               | 1,000          | 0.17 |
| Second  | Sodium thiosulfate | 970            | 0.08 |

This example shows that sulfur compounds, such as sodium thiosulfate, act as stabilizers in reducing the fog of emulsions sensitized with gold and activated non-labile selenium compounds.

## EXAMPLE 11

A coarse-grained silver bromoiodide emulsion containing 2.85 mole percent iodide is prepared and a first portion chemically sensitized with 2 mg. of gold sulfide per silver mole, 15 mg. of sodium thiocyanate per silver mole and 2.3 mg. of potassium selenocyanate per silver mole. This first portion of the emulsion is then digested for 25 minutes at 65° C. in the presence of 50 grams of an inert gelatin per silver mole.

A second portion of the emulsion is chemically sensitized and heated in the same manner as the first portion except that 50 grams per silver mole of a naturally active gelatin was utilized.

These portions of the emulsion are then coated and processed in the same manner as in Example 1 with the following results:

| Portion | Gelatin | Relative speed | Fog  |
|---------|---------|----------------|------|
| First   | Inert   | 100            | 0.16 |
| Second  | Active  | 118            | 0.22 |

This example illustrates the unpredictability connected with using potassium selenocyanate in combination with noble metals as a sensitizer with various gelatins. U.S. Patent 3,243,298, column 68, lines 35-38, and British Patent 861,984, page 2, lines 42-44 disclose the use of potassium selenocyanate as a sensitizer. There is no disclosure of the use of this compound in combination with noble metals, however, or that activation of this compound will give synergistic sensitizing results in combination with noble metals. The limited disclosure in these reference should thus be qualified as being dependent upon the type of gelatin employed. By employing the process of my invention, I can obtain reproducible results which are not dependent upon the particular type of gelatin employed.

## EXAMPLE 12

## Test for labile and non-labile selenium compounds

To 10 ml. of distilled water in a test tube is added 6 mg. of potassium selenocyanate. To this solution approximately 15 ml. of 0.1 N silver nitrate is added. No silver selenide is formed which indicates that potassium selenocyanate is a non-labile selenium compound.

To 10 ml. of distilled water in a test tube is added 6 mg. of potassium selenocyanate. To this solution is added 50 mg. of sodium sulfite. No reaction occurs. To this solution approximately 5 ml. of 0.1 N silver nitrate is added. A black precipitate (silver selenide) immediately forms. This indicates that the potassium selenocyanate becomes labile in the presence of sodium sulfite, a reducing agent.

In one embodiment of the present invention we employ a complex formed by gold salt with phosphine. This complex is not itself a sensitizer but it is added as a source of both gold salt as a sensitizer and phosphine as an activator for the non-labile selenium added separately. Triphenylphosphinegold (I) chloride is a well defined complex which has been isolated and purified. See Journ. Chem. Soc., 5751 (1965). When added to the emulsion

## 12

the complex dissociates liberating the gold salt and triphenylphosphine components.

## EXAMPLE 13

Lack of sensitizing ability of the complex by itself; lack of sensitizing ability of non-labile selenium by itself.

A medium grained silver bromoiodide emulsion containing 3.4 percent iodide was chemically sensitized with (per mole of silver halide) 4.75 mg. triphenylphosphinegold (I) chloride and 100 mg. sodium thiocyanate.

A second portion of the emulsion was sensitized with 100 mg. sodium thiocyanate and 1.4 mg. potassium selenocyanate.

A third portion was sensitized with 4 mg. potassium chloroaurate (equimolar amount of gold, compared to sample 1) and 100 mg. sodium thiocyanate.

Each of the three samples was heated for 40 minutes at 65° C.

These emulsion samples were then coated on a cellulose acetate support at a coverage of 540 mg. silver per square foot. The coatings were exposed on an intensity scale sensitometer, processed for 5 minutes in Kodak Developer DK-50, fixed, washed, and dried.

| Portion (description)                  | Relative speed | Fog  |
|----------------------------------------|----------------|------|
| First (phosphine-gold complex alone)   | <10            | 0.04 |
| Second (potassium selenocyanate alone) | <10            | 0.04 |
| Third (gold sensitizer alone)          | 100            | 0.05 |

## EXAMPLE 14

Activation of a non-labile selenium compound with the complex; simultaneous activation of the gold compound to produce a gold-sensitization

The emulsion of example 13 was chemically sensitized with (per mole of silver) 4.75 mg. triphenylphosphinegold (I) chloride, 100 mg. sodium thiocyanate, and 1.4 mg. potassium selenocyanate. The sample was heated for 40 minutes at 65° C.

A second portion of the emulsion was sensitized with 4 mg. potassium chloroaurate (equimolar to the amount of gold in portion 1), 100 mg. sodium thiocyanate, and 1.4 mg. potassium selenocyanate. The sample was heated for 40 minutes at 65° C.

A third portion of the emulsion was sensitized with 100 mg. sodium thiocyanate, 1.4 mg. potassium selenocyanate and 2.55 mg. triphenylphosphine (equimolar to the amount of phosphine in the complex of sample 1). This portion was heated 1 minute at 65° C.

These emulsion samples were coated, exposed, and processed as in Example 13.

| Portion (description)                  | Relative speed | Fog  |
|----------------------------------------|----------------|------|
| First (phosphine-gold complex + KSeCN) | 151            | 0.12 |
| Second (gold sensitizer + KSeCN)       | 100            | 0.07 |
| Third (phosphine + KSeCN)              | 74             | 0.13 |

In the above, the comparison of portions 1 and 2 illustrates the activation of non-labile selenium by the phosphine-gold complex (there is little or no activation of any kind in portion 2). The comparison of 1 with 3 illustrates that a gold sensitization also occurs in portion 1; non-labile selenium activated by a good "reducing compound," in the absence of gold produced a relative speed of only 74.

## EXAMPLE 15

## Inability of the complex to chemically sensitize with labile selenium

The emulsion of Example 13 was chemically sensitized with (per mole of silver) 4 mg. of potassium chloroaurate, 100 mg. sodium thiocyanate, and 1.45 mg. N,N-dimethylselenourea. The portion was heated for 5 minutes at 65° C.

A second portion was sensitized with 4.75 mg. triphenyl-

phosphine-gold (I) chloride, (equimolar in gold to the gold-sensitizer used in sample 1), 100 mg. sodium thiocyanate, and 1.45 mg. N,N-dimethylselenourea. This sample was heated for 20 minutes at 65° C.

The samples were coated, exposed, and processed as in Example 1.

| Portion (description)                           | Relative speed | Fog  |
|-------------------------------------------------|----------------|------|
| First (gold+selenium finish)                    | 100            | 0.49 |
| Second (phosphine-gold complex+labile Selenium) | 5.9            | 0.05 |

#### EXAMPLE 16

##### Equivalence of the method with sensitization by gold+labile selenium

A coarse grained silver bromoiodide emulsion containing 6 mole percent iodide was chemically sensitized with (per mole of silver) 2 mg. potassium chloraurate, 50 mg. sodium thiocyanate, 4 mg. sodium thiosulfate pentahydrate, and 0.5 mg. N,N-dimethylselenourea. The sample was heated for 5 minutes at 65° C.

A second portion was sensitized with 7.8 mg. triphenylphosphine-gold(I) chloride, 100 mg. sodium thiocyanate and 2.06 mg. Complex D.<sup>1</sup> The sample was heated for 25 minutes at 65° C.

A third portion of the emulsion was chemically sensitized with 7.8 mg. triphenylphosphine-gold(I) chloride, 100 mg. sodium thiocyanate and 1.8 mg. potassium selenocyanate. The sample was heated 20 minutes at 65° C.

The emulsion samples were then coated on a cellulose acetate support at a coverage of 540 mg. silver per square foot. The coatings were exposed on an intensity scale sensitometer, processed for 4 minutes in Kodak Developer D-19, fixed, washed, and dried.

| Portion (description)                                                 | Relative speed | Fog  |
|-----------------------------------------------------------------------|----------------|------|
| First (Optimum gold+labile selenium finish for this emulsion)         | 100            | 0.08 |
| Second (gold-phosphine complex+isoselenocyanate complex) <sup>1</sup> | 105            | 0.10 |
| Third (gold-phosphine complex+KSeCN)                                  | 95             | 0.08 |

<sup>1</sup> Complex D=[(CH<sub>3</sub>)<sub>4</sub>N]<sub>4</sub>[Co(NCSe)<sub>6</sub>].

Although the invention has been described in detail with reference to certain preferred embodiments thereof, variations and modifications can be effected within the spirit and scope of the invention as described hereinbefore and as defined in the appended claims.

I claim:

1. A process comprising sensitizing a photographic sil-

ver halide emulsion with a sensitizing amount of a noble metal and labile selenium, said labile selenium being formed in situ by activating a non-labile selenium compound.

- 5 2. The process of claim 1 wherein said non-labile selenium compound is activated by a reducing agent.
3. The process of claim 1 wherein said noble metal is gold.
4. The process of claim 2 wherein said noble metal is gold.
5. The process of claim 1 wherein said non-labile selenium compound is either potassium selenocyanate or selenous acid.
- 15 6. The process of claim 3 wherein said non-labile selenium compound is either potassium selenocyanate or selenous acid.
7. The process of claim 4 wherein said non-labile selenium compound is potassium selenocyanate or selenous acid.
- 20 8. The process of claim 2 wherein said reducing agent is a benzothiazolium salt, 2-mercaptopbenzoic acid, triphenylphosphine, stannous chloride or an alkali metal sulfite.
- 25 9. The process of claim 4 wherein said reducing agent is a benzothiazolium salt, 2-mercaptopbenzoic acid, triphenylphosphine, stannous chloride or an alkali metal sulfite.
- 30 10. The process of claim 7 wherein said reducing agent is a benzothiazolium salt, 2-mercaptopbenzoic acid, triphenylphosphine, stannous chloride or an alkali metal sulfite.
11. The process of claim 1 wherein said sensitizing is carried out in the presence of a water-soluble thiocyanate compound.
- 35 12. The process of claim 4 wherein said sensitizing is carried out in the presence of a water-soluble thiocyanate compound.
13. The process of claim 1 wherein said silver halide emulsion is stabilized with a labile sulfur compound.
- 40 14. The process of claim 4 wherein said silver halide emulsion is stabilized with a labile sulfur compound.
15. The process of claim 11 wherein said silver halide emulsion is stabilized with a labile sulfur compound.

#### References Cited

##### UNITED STATES PATENTS

- 3,297,446 1/1967 Dunn ----- 96-107  
 3,297,447 1/1967 McVeigh ----- 96-107 X

50 NORMAN G. TORCHIN, *Primary Examiner.*

RICHARD E. FICHTER, *Assistant Examiner.*